

G. E. DUNTON.

METHOD OF BACKING UP ELECTROTYPE SHELLS IN THE MANUFACTURE OF ELECTROTYPE PLATES.  
APPLICATION FILED JUNE 24, 1911.

1,073,105.

Patented Sept. 16, 1913.

Fig. 1.



Fig. 2.



WITNESSES

E. C. Tate  
M. J. Donegan

INVENTOR  
George E. Dunton  
by Blackwood Bros.,  
Attorneys.

# UNITED STATES PATENT OFFICE.

GEORGE E. DUNTON, OF NEW YORK, N. Y.

## METHOD OF BACKING UP ELECTROTYPE-SHELLS IN THE MANUFACTURE OF ELECTRO-TYPE-PLATES.

1,073,105.

Specification of Letters Patent. Patented Sept. 16, 1913.

Application filed June 24, 1911. Serial No. 635,195.

To all whom it may concern:

Be it known that I, GEORGE E. DUNTON, residing at New York, in the county of New York and State of New York, a citizen of the United States, have invented certain new and useful Improvements in Methods of Backing up Electrotype-Shells in the Manufacture of Electrotype-Plates; and I do hereby declare the following to be a full, clear, and exact description of the invention, such as will enable others skilled in the art to which it pertains to make and use the same.

My invention relates to an improved method of backing up electrotype shells in the manufacture of electrotype plates.

It has for its object the uniting of metals, or other materials, having different melting points into a composite body, particularly to form a backing on a printing shell.

The invention consists in taking a metal, which has been previously formed in the shape of a printing shell, and placing it in an open receptacle, preferably a backing pan, treating the back of the shell with a binding substance, heating the open receptacle, shell and the binding substance thereon, closing and sealing the receptacle, heating the closed receptacle and shell and finally forcing the molten metal which is to form the backing of the shell, into the closed receptacle under continuous pressure so that all the molten metal necessary to completely fill all the indentures or interstices formed in the shell, by the letters or other characters, will be forced in before any of the molten metal becomes set and then allow the shell and its backing to set and cool, while still under pressure, thus causing the backing to be firmly united to the shell and form therewith a composite body.

The metal above referred to, which is formed in the shape of a printing shell, is made preferably of copper but may be made of nickel, steel, brass or any other suitable metal having a melting point higher than the metal with which it is to be combined or joined to form a backing therefor. The other metal above referred to, which is to be joined to the back of a printing shell and form a backing therefor, is composed preferably of a combination of lead, tin and antimony in about the following proportions: lead, 96 per cent.; tin, 2 per cent. and antimony, 2 per cent.

The melting point of electrolytic copper, of which the printing shell is made, is about 2550 degrees Fahrenheit, the melting point of the solder or binder which is applied to said shell, is about 530 degrees Fahrenheit and the metal which is united to said copper shell through the medium of the melted binder and forms a backing for said shell attains a molten state at about 625 degrees Fahrenheit.

In the drawings, which illustrate one form of apparatus for carrying out my method:—Figure 1 is a sectional view of the receptacle or backing pan and printing shell with the binder applied. Fig. 2 is a side elevation of the receptacle or backing pan with the cover thereon locked and sealed, the backing pan, printing shell, binder and molten metal backing being shown in dotted lines.

Referring to the drawings in which like reference characters denote like parts throughout the several views, 1 represents the receptacle or backing pan adapted to be mounted on set screws 2, to provide means for leveling the same, and 3 is the cover which when applied to the receptacle and locked thereon forms a sealed closure. The means for locking and sealing the cover to the receptacle or backing pan consists of pivoted clamps 4. The molten metal backing is introduced into the sealed closure by means of a nipple or short pipe 5, one end of which is inserted into an orifice 6, formed in the cover and receptacle, and the opposite end connected to a suitable pump situated on or in the melting pot of a furnace. The printing shell is represented at 7, the solder or binder at 8 and the molten metal backing at 9.

Ordinarily in uniting or joining one metal to another, in a cold state, it is possible to place tin or solder foil between the two surfaces to be joined, bind the metals together, apply pressure and heat both until the tin or solder foil melts and adheres to the surfaces of both metals and binds the said metals together and upon becoming cooled to the temperature of the surrounding atmosphere, said metals are hermetically joined one to the other.

In the "backing up" of an electrotype shell, which comprises the joining of the backing metal to the electrotype shell, it is impossible to proceed as above described as

the shell is very delicate as it varies in thickness from one one thousandth to five one thousandths of an inch and the surface is uneven, caused by numerous indentures or interstices in its back which conform to the general contour of its face or surface, in reverse, and if sufficient pressure were applied to insure the forcing of the solder or other binding substance together with the metal comprising the backing, in a cold or rigid state, into the indentures or interstices, the elevated portions or projections, forming the back of the electrotype shell, would be forced into the face of the shell and crush it and the entire shell would be ruined. It will also be seen that in order to have the types and other printing surfaces withstand the pressure which it is necessary to apply to the electrotype plate during the process of printing, which sometimes calls for hundreds of thousands of impressions from the surface of a printing plate, the backing must fill up all the recesses in the back of the shell, which are behind or underneath the faces of the letters or other printing surfaces, and be made to conform to the general contour of the face of the shell along the line of junction at the back, without crushing in the elevations on the back, which are the spaces between the types on the printing surface which is the face of the electrotype plate. The final surface of the back which has been joined to the electrotype shell must have an even, flat, perfectly level surface, and all parts be in a plane perfectly parallel to that of the printing surface of the electrotype plate.

In the practice of my method, I first produce the metallic electrotype shell, which may be made of copper, steel, nickel or other suitable material, in the usual manner, by the electrodeposition of the desired metal upon the conductive surface of a prepared wax mold, although a mold of lead or other suitable material would serve the same purpose, and having secured the desired thickness for the shell, I remove the shell from the surface of the wax mold by pouring boiling hot water over the surface of the shell which heats the metal and breaks the adhesion between the wax of the mold and the metal of the shell, when the shell can be easily stripped off and pulled away from the mold, then I rinse the shell in boiling hot lye, to remove all traces of wax which may have adhered thereto, and then plunge the said shell into a pickle composed preferably of sulfuric acid and water to remove all traces of the lye, and after thoroughly rinsing in running water the shell is reasonably clean and ready for the application of the backing. I then take one of the metals, preferably in the shape of an electrotype shell and treat said shell with a soldering flux solution, composed of ammoniated mu-

riate of zinc dissolved in water, by washing the back surface well with said solution and allowing the surplus liquid to drain off, then place the shell, treated as above described, in the open receptacle, or backing pan, and apply the soldering foil or cement binder over the back surface of the shell and cause said soldering foil or binder to adhere to the said treated surface on the back of the shell by subjecting the open receptacle and the shell therein to a degree of heat sufficient, or more than sufficient, to melt the soldering foil or binder and cause it to run into all the indentures or interstices in the back surface of the shell and completely cover said back surface. The said open receptacle and the shell therein are heated, preferably, by placing the receptacle in the melting pot containing molten metal and allowing it to float on the surface of the said molten metal until the shell becomes heated to the desired degree, after which the receptacle and shell are removed from the melting pot and placed on a suitable stand. The cover which has been previously heated in any desired manner, is then applied to the receptacle and clamped and sealed thereon by means of suitable clamps and thereby, in combination with the receptacle or backing pan forms a closure, molten metal, which is to form the backing for the shell, is then forced through the nipple or short pipe by a pump or other means into the interior of the closure and over the back surface of the shell, which as before stated has been previously treated with a soldering flux solution and soldering foil and heated, and said molten metal fills all of the interstices or indentations in said shell and also completely fills the closure, then the closure and its contents are cooled, by any suitable means, and allowed to set and thus form a composite body after which the shell with the backing firmly united therewith and forming a printing plate is sawed into the desired sizes and finished in the usual well known manner to fit it for use in printing.

As the metal cools, it will contract or shrink and to compensate for such contracting or shrinkage the pressure by the pump on the molten metal is constantly maintained, which causes the molten metal to continuously flow into the closure and fill up any space caused by contraction or shrinkage before the metal has set and keeps the closure full at all times.

What I claim is:—

1. The method of forming a composite body, consisting in taking two metals one of which is in the shape of a printing shell and melts at a high temperature and the other to form the backing for the shell and melting at a low temperature, applying a binder to the shell, placing the shell in a receptacle, forming a closure by applying

70

75

80

85

90

95

100

105

110

115

120

125

130

- a cover to the receptacle, maintaining a substantially constant air tight closure while the cover is in place, heating the closure and the shell therein until the binder melts,  
5 introducing molten metal into the closure and causing it to fill the closure and the interstices in the shell and breaking the substantially air tight closure by removing the cover, substantially as described.  
10 2. The method of forming a composite body, consisting in taking two metals one of which is in the shape of a printing shell and melts at a high temperature and the other to form the backing for the shell and  
15 melting at a low temperature, applying a binder to the shell, placing the shell in a re-

ceptacle, forming a closure by applying an air tight cover to the receptacle, maintaining a substantially air tight closure while the cover is in place, heating the closure 20 and the shell therein until the binder melts, introducing molten metal into the closure and causing it to fill the closure and the interstices in the shell and breaking the substantially air tight closure by removing the 25 cover, substantially as described.

In testimony whereof, I affix my signature in the presence of two witnesses.

GEORGE E. DUNTON.

Witnesses:

FRANCIS S. DUFF,  
H. BECKER.